

Ordinary Soap 300

S-31

Hyposulphite of Soda  
Borax  
Spirits of Ammonia

## UNITED STATES PATENT OFFICE.

CHARLES F. BROADBENT, OF BALTIMORE, MARYLAND.

SOAP.

SPECIFICATION forming part of Letters Patent No. 292,980, dated February 5, 1884.

Application filed December 11, 1883. (No specimens.)

To all whom it may concern:

Be it known that I, CHARLES F. BROADBENT, of the city of Baltimore and State of Maryland, have invented certain Improvements in Soap, of which the following is a specification.

In carrying out my invention I take of ordinary soap ten (10) pounds and dissolve it in five (5) gallons of water, to which has been previously added two and one-half (2½) pounds of hyposulphite of soda and three (3) ounces of borax. To this mixture is then added two and one-half (2½) ounces of spirits of ammonia, and, if necessary, two (2) ounces of common salt. The mixture is then boiled, and while hot poured into molds, in which it is

allowed to cool. This soap is found to possess superior detergent qualities, is cheaper than ordinary soap, and will not injure the hands.

I do not limit myself to the exact proportions of the various ingredients herein specified or to the employment of common salt; but

I claim as my invention—

An improved soap, which consists of ordinary soap, water, hyposulphite of soda, borax, and spirits of ammonia, all combined substantially as specified.

CHARLES F. BROADBENT.

Witnesses:

WM. T. HOWARD,  
CHAS. B. CASSADY.

NG H 502